

## UNITED STATES PATENT OFFICE

MILTON O. SCHUR AND BENJAMIN G. HOOS, OF BERLIN, NEW HAMPSHIRE, ASSIGNEES  
TO BROWN COMPANY, OF BERLIN, NEW HAMPSHIRE, A CORPORATION OF MAINE

## PRETREATMENT OF CELLULOSE PRIOR TO NITRATION

No Drawing.

Application filed March 19, 1929. Serial No. 348,357.

This invention relates to the preparation of nitrocelluloses and has for its object to provide a process of conditioning cellulose fiber to render it more satisfactory for use as a raw material for the preparation of nitrocelluloses such as those employed in the manufacture of films, lacquers, artificial silk, and kindred products.

In U. S. Patent No. 1,701,543, issued February 12, 1929, to George A. Richter, Milton O. Schur, and Royal H. Rasch, the advantages of treating the fiber with solutions of nitrocellulose in organic solvents prior to nitration are disclosed. It is there stated that the characteristics of the fiber for nitration are markedly improved, as attested by the good quality of the nitrated product and by the higher yield and lower acid retention of the product. A drawback to the commercial application of the process therein disclosed, however, is the fire hazard associated therewith and the high cost of nitrocellulose solvents the loss of which makes the expense of conditioning the fiber excessive.

In accordance with the process of the present invention, the fiber is conditioned for nitration by treating with nitrocellulose dispersed in water, as we have found that beneficial results comparable to those obtained by the use of organic solvent solutions may be procured. Water thus serves as a vehicle or carrier for the nitrocellulose, in lieu of organic solvent, making the conditioning treatment far more economical and greatly reducing the fire hazard. The fiber is preferably dried before nitration, so as to avoid dilution of the nitrating acids.

While not restricted thereto, the process of the present invention may be applied to especial advantage in the case of wood pulp, as such fiber offers good opportunity for improvement. What we have in mind more particularly is a wood pulp of high alpha cellulose content which may be used as a cotton fiber substitute for the preparation of nitrocelluloses. Such pulp, however, under some circumstances may not be convertible into the nitrate with as high a yield as cotton fiber. By the process of the present invention, however, such fiber may be so modi-

fied in its characteristics that its yield upon nitration is raised. Apparently, the advantages gained result from the thin coating or film of nitrocellulose produced on the fibers, which, as fully described in the application hereinbefore identified, properly regulates the rate of nitration.

A treatment such as hereinbefore described may be practised advantageously when using pulp of various origins and in beaten, un-beaten, bulk, or sheeted condition. When pulp in bulk condition is treated with an aqueous dispersion of nitrocellulose, precipitation of the nitrocellulose may be effected as by the addition of a suitable precipitating agent, to fix the nitrocellulose on the fibers, whereupon the pulp may be sheeted into paper and the paper then nitrated. Under some conditions, however, it may be more expedient to treat the pulp in the form of waterleaf paper, and in such case the treatment may be readily carried out continuously and the treated paper then dried continuously, whereupon the dry paper may be nitrated. Nitration may be performed by passing the treated paper in the form of a continuous sheet through a bath of nitrating acid, or the sheet may be shredded or cut into small pieces and nitration effected in pots, as is customarily done.

The amount of nitrocellulose necessary to improve the fiber for nitration is very small, less than 1% affording a noteworthy gain in yield and lowering of acid retention. The aqueous dispersion of nitrocellulose may be prepared in any suitable manner known to those skilled in the art. For instance, as is known, the aqueous dispersion of nitrocellulose may be produced by initially forming a fairly concentrated solution of low-viscosity nitrocellulose in a suitable organic solvent, such as amyl acetate, and then mixing the solution with a comparatively large amount of water containing a small amount of stabilizer or dispersing agent, such as soap, to keep the dispersed nitrocellulose from precipitating out. A procedure answering this general description appears in British Patent No. 233,367, granted November 6, 1922, to T. Whittelsey. The aqueous dispersion of ni-

5 trocellulose may be applied to pulp in any suitable condition, in some cases it perhaps being advantageous to add dispersed high-boiling nitrocellulose solvents to the dispersion, containing a stabilizer such as a trace of soap, which may be necessary to keep the nitrocellulose from precipitating.

10 For example, a wood pulp of high alpha cellulose content in the form of waterleaf tissue of 30 pounds basis weight was passed through an aqueous dispersion of nitrocellulose, then squeezed free of excess liquid, dried, and nitrated in the usual way, using a nitrating acid consisting of 20.5%  $\text{HNO}_3$ , 60.8% 15  $\text{H}_2\text{SO}_4$ , 18.7%  $\text{H}_2\text{O}$ , the ratio of acid to fiber used being 50 to 1. The nitration was carried out at 40° C. for 30 minutes. Following are typical results that have been obtained according to this procedure, compared with the results from untreated paper:

|                                        | Untreated paper | Treated paper |
|----------------------------------------|-----------------|---------------|
| 25 Per cent nitrocellulose in paper    | 0               | 0.2           |
| Yield                                  | 150.7           | 154.5         |
| Initial temperature rise               | 1.6° C.         | 1.4° C.       |
| Acid retention                         | 3.6             | 3.5           |
| Color of nitrocellulose                | 21              | 20            |
| Nitrogen content of nitrocellulose     | 11.00           | 11.06         |
| Per cent of theoretical yield obtained | 97.4            | 99.5          |

30 From the table hereinbefore given, it is thus seen that the yield of nitrocellulose is notably increased, while the acid retention is reduced. The product was also slightly better in other characteristics than the product 35 from untreated paper.

An important advantage of the process herein described is that an aqueous medium serves as the vehicle or carrier for the nitrocellulose, it thus being possible to treat the 40 fibers uniformly with a thin coating or film of nitrocellulose at comparatively low expense.

Having thus described certain embodiments of this invention, it should be evident to those skilled in the art that various 45 changes and modifications might be made therein without departing from the spirit or scope of invention as defined by the appended claims.

We claim:

- 50 1. A process which comprises treating cellulose fiber with an aqueous dispersion of nitrocellulose, and then nitrating the fiber.
2. A process which comprises treating cellulose fiber with an aqueous dispersion of nitrocellulose, drying, and then nitrating the fiber.
- 55 3. A process which comprises treating cellulose fiber with an aqueous dispersion of nitrocellulose containing a stabilizer, and then nitrating the fiber.
4. A process which comprises treating cellulose fiber with a dispersion of nitrocellulose in a water-organic solvent mixture, and then nitrating the fiber.
- 60 5. A process which comprises treating cel-

lulose fiber with a dispersion of nitrocellulose in a water-organic solvent mixture containing a stabilizer, and then nitrating the fiber.

6. A process which comprises treating 70 paper with an aqueous dispersion of nitrocellulose, and then nitrating the paper.

7. A process which comprises treating paper with an aqueous dispersion of nitrocellulose, drying, and then nitrating.

8. A process which comprises treating 75 wood pulp with an aqueous dispersion of nitrocellulose, and then nitrating the pulp.

9. A process which comprises treating pulp with an aqueous dispersion of nitrocelluloses, fixing the nitrocellulose on the 80 fibers, sheeting into paper, and nitrating the paper.

10. Cellulose fiber containing previously dispersed nitrocellulose distributed therethrough and fixed thereon but otherwise 85 being in an unsized and unfilled condition.

11. A wood fiber of high alpha cellulose content containing previously-dispersed nitrocellulose in small amount distributed therethrough and fixed thereon but otherwise 90 being in an unsized and unfilled condition.

12. A waterleaf paper containing previously-dispersed nitrocellulose distributed through the pores and interstices thereof.

13. A waterleaf paper of wood fiber of 95 high alpha cellulose content containing previously-dispersed nitrocellulose in small amount distributed therethrough and fixed on the fibers.

In testimony whereof we have affixed our 100 signatures.

MILTON O. SCHUR.  
BENJAMIN G. HOOS.

105

110

115

120

125

130